

## UNITED STATES PATENT OFFICE

2,070,901

## METHOD OF DEOXIDATION CONTROL

Anson Hayes and Jesse J. Canfield, Middletown, Ohio, assignors to The American Rolling Mill Company, Middletown, Ohio, a corporation of Ohio

No Drawing. Application November 12, 1931,  
Serial No. 574,676. Renewed January 24, 1934

3 Claims. (Cl. 23—230)

Our invention relates to methods of control of deoxidation in the manufacture of iron and steel. In the past it has been the practice in the manufacture of iron and steel, to add deoxidizing materials to the metal bath pursuant to a rule of thumb practice, which has no real accuracy. It has been attempted to govern the amount of deoxidizing substance by attempting to follow a uniform practice in the refining of the metal charge, 5 and then adding a measured and uniform quantity of deoxidizer per ton of metal. It has been attempted to judge the oxide content of a bath of iron or steel by an examination of the slag, and by an observation of the conditions in the 10 furnace and of the fracture of a sample, etc.

None of these methods are accurate, and particularly when expensive substances are added to a metal bath, which substances are readily oxidizable, it is necessary to know just how much to 15 add or else there will be wastage, or over or under use of the particular material.

If it were possible to attain it, a true analysis 20 of the oxide content of a bath of steel or iron is the only way in which to govern accurately the amount of addition of oxidizable substances which 25 may be or are required to be added thereto. The difficulty with following such a practice is that until our invention, which we now propose to describe, the determination of oxide content of 30 molten metal was a long and delicate task taking hours in the laboratory, and it is obvious that in the making of iron and steel there can be no extended wait in the process after the metal is finished and before tapping, or otherwise treating 35 the metal, so that such an analysis could be made.

We have discovered a mode of analysis for oxygen content in molten iron and steel which can be completed in twenty minutes or less, and is not a delicate or difficult operation at all, and hence 40 our invention relates to the control of oxidizable additions to a completed body of iron and steel by a test of the oxide content of the metal itself, carried out by chemical analysis, and preferably according to the steps which we will now outline.

45 When the refining procedure is substantially complete and the metal is in the condition requiring tapping or deoxidizing, we take a sample of the metal from beneath the slag, this sample being a definite amount, and to this sample we 50 add a predetermined quantity of aluminum, which aluminum is considerably in excess of the amount which will chemically combine with all the possible oxygen in the metal. A convenient weight of drillings is taken from the product of this re- 55 action after cooling the same, and the material,

other than aluminum oxide, is dissolved away. This can be done with a solution of iodine. The iodine solution when heated attacks and quite readily and quickly dissolves the iron and other metals including aluminum, but does not attack 5 aluminum oxide (alumina). When the iron has been dissolved off (and the remaining, which is alumina residue plus carbon is washed and ignited to dry it and drive off carbon), the remaining material, which is alumina, is weighed. By the formula  $Al_2O_3$  and atomic weights of these two elements, the exact weight of the oxygen which was in the drilling is obtained. From this may be obtained the percentage of oxygen present in the drillings and therefore also in the original bath 15 of iron or steel.

The whole procedure can be completed in less than twenty minutes, and the oxide content will not be materially increased by holding the bath for such a short period; nor will the ability to tap 20 the metal properly and at proper temperature be interfered with.

While the described iodine method seems to be 25 the most suitable because of its rapidity, other dissolving agents may be used giving comparatively quick results, to wit, nitric acid, nitric acid mixed with hydrochloric acid, salts mixed with acids, mixtures of acids with an oxidizing agent in which a halogen is set free.

A method using cold nitric acid which we have 30 successfully employed is as follows:

The sample is prepared for analyses by the same practice used in the iodine method. Ten grams of the sample are dissolved with 200 m. l. of dilute nitric acid (1.2) in a beaker of sufficient 35 size to eliminate any loss of sample due to violent effervescence during solution of the sample. The acid is added carefully to prevent a reaction which is too violent. When the sample is in solution, one hundred and fifty m. l. of cold water 40 are added and the solution is filtered immediately on a fairly retentive filter paper, using suction apparatus if necessary. The residue remaining on the paper is washed first with hot water and then alternately with hot dilute hydrochloric acid (1—1) and water until free from iron salts. The filter paper and residue are transferred to 45 a weighed platinum crucible and ignited to remove the paper and other carbonaceous material. The crucible is weighed. Difference in weight 50 represents aluminum oxide. The oxygen in the aluminum oxide is calculated to per cent oxygen in the material under test and serves as a guide for proper deoxidation.

In this manner we are able to control the 55

amount of substance to be added with exact relationship to the amount of oxygen in the metal to which it is to be added. The addition may be made in accordance with any accepted practice.

5 It will naturally be possible to use another substance than aluminum, which has a like property of combining with oxygen to make an oxide which resists the action of solvents which will quickly dissolve iron or steel. If an alloy of 10 iron or steel is the product of the finished metal bath and any of the ingredients are insoluble in the iron solvent employed, then allowance will have to be made for them, if the alloying metals are in any amount which would interfere with 15 reaching a sufficiently accurate percentage.

While we have described our new process in connection with iron and steel, it may be also employed in the deoxidation of other metals such as, for instance, copper and brass.

20 Having thus described our invention, what we claim as new and desire to secure by Letters Patent, is:—

1. A process for the treatment of iron or steel which comprises refining the iron or steel in 25 the usual way and at the conclusion of the refining process and while maintaining the bath of metal molten, chemically determining the percentage of oxygen therein by taking a determined sample of the material, combining it with an 30 amount of aluminum which is in excess of any amount necessary to combine with the oxygen present in the sample by chemical combining weight, then dissolving the iron or steel from the sample, or part thereof of a determined weight, 35 without affecting the alumina, and finally weighing the remaining solid and calculating the weight of oxygen and hence its percentage in the metal sample and the amount of deoxidizer necessary to bring said metal bath to a desired state of de-

oxidation, all of said steps being carried on rapidly while said metal bath is maintained molten and in a condition for deoxidation, and then adding deoxidizing agent to said metal bath as determined by said calculation.

5 2. That method of determining the oxygen content of a mass of molten iron or steel which consists in combining a determined sample with an amount of aluminum which is in excess of an amount necessary by chemical combining 10 weights to combine with the probable oxygen present in the sample, then rapidly dissolving the iron or steel from the sample or a weighed portion, without affecting the alumina and finally weighing the remaining alumina, calculating the 15 weight of oxygen therein and comparing this with the weight of the sample portion, whereby to determine the oxygen content of said mass of molten iron or steel, all of said steps being carried on so rapidly that said determination can 20 be made between the conclusion of the refining process for said metal and the deoxidation of the same metal.

3. That method of determining the oxygen content of a mass of molten iron or steel which consists in combining a determined sample with an amount of aluminum which is in excess of an amount necessary by chemical combining weights to combine with the probable oxygen present in the sample, then dissolving the iron or steel from 25 the sample, or a weighed portion thereof, without affecting the alumina, and finally weighing the remaining alumina, calculating the weight of oxygen therein and comparing this with the weight of the sample portion, said dissolving action being accomplished by the use of hot iodine 30 solution as a solvent.

ANSON HAYES.  
JESSE J. CANFIELD.